

1

3,280,029

## LUBRICANT COMPOSITIONS

Hans F. Waldmann, Glassboro, N.J., assignor to Mobil Oil Corporation, a corporation of New York  
No Drawing. Filed June 18, 1964, Ser. No. 376,249  
21 Claims. (Cl. 252—49.5)

The present invention is directed to lubricant compositions possessing improved characteristics. More particularly, it is directed to improved lubricating oils and water-in-oil emulsions.

The vapor phase corrosion or rusting of metal parts is often an acute problem in machines or systems which contain water. Such corrosion most frequently occurs at the metal surfaces enclosing vapor spaces, and is a particular problem in systems which employ water-in-oil emulsions such as hydraulic fluids as functional fluids for transmitting mechanical energy. Indeed, although water-in-oil emulsions are widely used today as lubricants and functional fluids, this problem of vapor phase corrosion is a major drawback to their more widespread use particularly as functional fluids for power transmission and the like.

Due to the more rigorous demands of modern technology, increasing attention is being given to the problem of fatigue in metal components which are subject to repeated stress. Such metal fatigue is also a particular problem in systems employing water-in-oil emulsions as functional fluids. The metal components in such systems frequently tend to be subject to early fatigue failures. For example, due to the fatigue failure of bearings, the useful life of gear pumps employing water-in-oil emulsions is often only about one-fifth as great as that of gear pumps which employ other types of functional fluids.

In accordance with the present invention, I have found that by incorporating a specific type of compound into lubricant compositions, it is possible to provide compositions which are capable of imparting effective and long-lasting vapor phase corrosion resistance, improved anti-fatigue qualities and other desirable characteristics.

It is therefore an object of the present invention to provide improved lubricants. A further object is to provide a method for improving the characteristics of such lubricants. Another object is a method for enhancing the vapor phase corrosion resistance and anti-fatigue characteristics of metals which are subject to conditions which promote vapor phase corrosion and metal fatigue. A further object is to provide effective additives for lubricants. A particular object of the present invention is to provide water-in-oil emulsions exhibiting superior characteristics especially vapor phase corrosion resistance and anti-fatigue characteristics. Other objects of the invention as well as some additional advantages thereof will become apparent hereinafter.

The foregoing and other objects are achieved by incorporating into the lubricants certain alkyl amino mono-alkanols possessing the general formula:



where

R represents an alkyl group;

R' represents an alkyl group the same or different from R, or a hydrogen atom; R and R' are selected so that

2

sum of the groups represented by R+R' does not exceed 10 carbon atoms; X is an alkylene group having from 2 to about 4 carbon atoms; and

5 n is 1 or 2.

The alkyl groups present in these amine compounds may be either straight or branched-chain; primary, secondary or tertiary alkyls so long as the combined total of carbon atoms does not exceed ten. Similarly, the alkylene groups represented by X may be straight or branched-chain and can be derived from either primary, secondary or tertiary alkyls.

It will be seen from the above general formula that the compounds encompassed thereby may be characterized as monoalkyl or dialkyl amino mono-alkanols or alkoxy mono-alkanols. Some examples of such compounds include: monomethyl amino ethanol, dimethyl amino ethanol, monoethyl amino ethanol, monoethyl amino ethoxy ethanol, diethyl amino ethanol, diethyl amino ethoxy ethanol, diisopropyl amino ethanol, dibutyl amino ethanol, dibutyl amino ethoxy ethanol, n-butyl amino ethanol, dimethylamino-2-propanol, diisopropyl amino 2-propanol, n-butyl amino 2-propanol, isobutyl amino 2-propanol, dimethyl amino 2-butanol, dimethyl amino 1-butanol, etc.

The alkyl amino mono-alkanol compounds described herein may be advantageously employed in a variety of liquid lubricant compositions. They are particularly effective in liquid lubricant compositions which contain water as a component or impurity, or in liquid lubricants employed in machines, apparatus or systems which are subject to conditions which promote vapor phase corrosion and/or metal fatigue either in the presence or absence of water.

35 Some examples of such liquid lubricants include mineral oil or synthetic oil-based lubricating oil compositions suitable for use as automotive lubricants such as motor oils, gear oils and the like; aviation lubricants including jet engine oils; marine lubricants such as marine diesel oils; industrial lubes as exemplified by metal working oils, gear oils; and the like. Also included are the single phase lubricating compositions or functional fluids containing water and a synthetic base oil such as the glycol fluids containing water, glycols and polyglycols.

40 Further examples of liquid lubricants which may be improved in accordance with the invention include water-in-oil emulsions such as those employed as metal working fluids, oven chain lubricants, as well as those used as functional fluids such as hydraulic fluids, transmission fluids etc. Indeed, the use of the aforescribed mono-alkanol compounds with water-in-oil emulsions is a particular aspect of the present invention. It has been found that the instant mono-alkanol compounds because of their alkaline character are compatible with and particularly effective in water-in-oil emulsions which possess an alkaline or in some cases neutral environment. This is in contrast to behavior of heretofore known acidic inhibitors which tend to precipitate out of the alkaline emulsions. 45 By employing the instant alkyl amino mono-alkanols it has been found that it is possible to impart to the emulsions not only vapor phase corrosion resistance and anti-fatigue properties, but also improved anti-wear characteristics and increased periods of useful life.

50 The above-described liquid lubricants, both lubricating oils and water-in-oil emulsions, may contain base oils of lubricating oil viscosity having widely varying origin and characteristics. Some examples of base oils include mineral oils from different crudes, i.e., naphthenic, paraffinic, etc.; which have been solvent and acid refined, hydro-cracked etc.; and synthetic oils such as olefin polymers, hydrogenated olefin polymers, alkylene oxide polymers,

dicarboxylic acid esters, liquid esters of phosphorus, monomeric and polymeric silicones, esters of polyhydroxy alcohols and the like.

In the case of water-in-oil emulsions the base oil and water may be employed in various relative proportions, the water being present generally in the range from about 10 to 70% by weight of the emulsion. Water-in-oil emulsions containing hydrocarbon base oils of from about 50-400 S.U.V. at 100° F. are of particular interest.

The use of the particular alkyl amino mono-alkanol compounds defined hereinabove is necessary in order to achieve the desired vapor phase rust resistance, anti-fatigue properties and other desirable characteristics. The structure and characteristics of these specific mono-alkanol compounds is important for it has been found, as will be shown hereinafter, that similar compounds including alkyl amines and certain di-alkanol compounds are not as effective in lubricant compositions. It should also be noted that the instant alkyl amino mono-alkanols must be present in the lubricant in an effective state. The mono-alkanol compound should be free to act in the lubricant composition. This invention therefore should be distinguished from the use of reaction products, complexes or the like of the mono-alkanol compounds with other components wherein the mono-alkanols would be tied up or otherwise have their effectiveness diminished or destroyed.

The superiority of the lubricant compositions of the present invention containing the aforescribed alkyl amino mono-alkanol compounds will be seen from the following series of comparative tests.

#### Vapor phase anti-rust test

This test measures the effectiveness of various amino compounds as vapor phase rust inhibitors in lubricants. According to the test procedure, a 16 ounce tallform widemouth glass jar is half filled with the fluid to be tested. A sandblasted and solvent-cleaned steel test panel is attached to the inside of a tin lid with a magnet and the lid then screwed loosely onto the glass jar to allow some "breathing." The jar is then immersed overnight up to the fluid level in a water bath maintained at 175° F. and during the day removed and stored at room temperature for 8 hours. The vapor phase anti-rust capability of the fluid is determined by measuring the percent of test panel surface rusted after various periods of exposure. The smaller percent of rusting the more effective is the inhibitor.

The results obtained with a water-in-oil emulsion after 7 days of exposure to test conditions is reported in Table 1, while the test results obtained after test periods of 27, 38 and 70 days is reported in Table 2.

The isopropyl amino ethanol employed in the following tests is, unless otherwise indicated, a commercial product containing about 60% of isopropyl amino ethanol.

TABLE 1.—VAPOR PHASE ANTI-RUST TEST

| Test No.       | Inhibitor              | Weight Percent | Percent Panel Surface Rust After 7 Days |
|----------------|------------------------|----------------|-----------------------------------------|
| 1 <sup>1</sup> | Isopropylamino ethanol | 0.1            | 100                                     |
| 2              | Morpholine             | 0.1            | 5                                       |
| 3              | Diethylhydroxylamine   | 0.1            | 45                                      |
| 4              | Monoethanolamine       | 0.1            | 45                                      |
| 5              | Isopropylamino ethanol | 0.04           | 9                                       |
| 6              | Diethylhydroxylamine   | 0.04           | 80                                      |
| 7              | Butylamine             | 0.02           | 40                                      |
| 8              | Isopropylamine         | 0.02           | 93                                      |
| 9              | Isopropylamino ethanol | 0.2            | 0                                       |
| 10             | Monoethanol amine      | 0.2            | 45                                      |

<sup>1</sup> Commercial hydraulic fluid containing 52 wt. percent of a naphthenic oil having a S.U.V. of 100 at 100° F., and 40 wt. percent water.

TABLE 2.—VAPOR PHASE ANTI-RUST TEST

| Test No.       | Inhibitor              | Weight Percent | Percent Panel Surface Rust After |         |         |
|----------------|------------------------|----------------|----------------------------------|---------|---------|
|                |                        |                | 27 days                          | 38 days | 70 days |
| 1 <sup>1</sup> | Isopropylamino ethanol | 0.2            | 1                                | 1       | 1       |
| 2              | do                     | 0.3            | 0                                | 0       | 0       |
| 3              | Butylamine             | 0.1            | 5                                | 30      | 70      |
| 4              | do                     | 0.2            | 3                                | 25      | 60      |

<sup>1</sup> In commercial hydraulic fluid described in Table 1.

It will be noted from Table 1 that water-in-oil emulsions containing the instant alkyl amino alkanols (tests 2, 6 and 10) possessed excellent vapor phase anti-rust capabilities as evidenced by the low percent panel rusting. By contrast, the same water-in-oil emulsions containing a well known vapor phase rust inhibitor morpholine (test 3) and monoethanol amine (test 5) which is structurally similar to the instant inhibitors, exhibited poor anti-rust characteristics.

Similarly, it is seen from Table 2 that emulsions containing the instant vapor phase rust inhibitors (tests 1 and 2) exhibited long term anti-rust characteristics as shown by the absence of any increase in panel surface rusting with increasing test periods. On the other hand, the same emulsions containing butylamine (tests 3 and 4) exhibited drastically increased rusting as the test period was extended from 27 to 70 days.

That the use of the instant alkyl amino monoalkanols is critical in order to obtain water-in-oil emulsions possessing the desired superior characteristics is demonstrated by the results reported in the following Table 3 where the emulsions of this invention were compared with similar emulsions containing certain dialkanol amines. In this particular test the fluid was continuously exposed to temperatures of 240° F. for periods of 1, 2 and 7 days.

TABLE 3.—VAPOR PHASE ANTI-RUST TEST

| Test No.       | Inhibitor                     | Weight Percent | Percent of Panel Surface Rust After Continuous Exposure at 240° F. for |        |        |
|----------------|-------------------------------|----------------|------------------------------------------------------------------------|--------|--------|
|                |                               |                | 1 day                                                                  | 2 days | 7 days |
| 1 <sup>1</sup> | None                          |                | 95                                                                     |        |        |
| 2              | Diisopropylaminoethanol       | 0.3            | 2                                                                      | 2      | 2      |
| 3              | Butylaminoethanol             | 0.3            | 4                                                                      | 4      | 4      |
| 4              | Diethylaminooctoxyetha-<br>no | 0.3            | 30                                                                     | 30     | 30     |
| 5              | Dibutylaminoethanol           | 0.3            | 35                                                                     | 40     | 40     |
| 6              | Methylaminodiethanol          | 0.3            | 90                                                                     |        |        |
| 7              | Ethylaminodiethanol           | 0.3            | 90                                                                     |        |        |
| 8              | Isopropylaminodiethanol       | 0.3            | 90                                                                     |        |        |
| 9              | Butylaminodiethanol           | 0.3            | 95                                                                     |        |        |

<sup>1</sup> In the commercial hydraulic fluid described in Table 1.

It is seen from Table 3 that while the emulsions of the invention containing the instant alkyl amino mono-alkanols (tests 2-5) exhibit superior and prolonged anti-rust properties, the emulsions containing the dialkanol compounds (tests 6-9) showed poor anti-rust capabilities and the test panels exposed to these latter emulsions were highly rusted after only one day of exposure.

Vapor phase anti-rust tests were conducted for more extended periods of time (up to 100 days) on several types of water-in-oil emulsions and lubricating oils as reported in Table 4. In this series of tests, water was added to each of the lubricating oil compositions and to the premium hydraulic fluid in the amounts shown in the table. The test procedure employed described above was used but the jar was immersed in a water bath maintained at 180° F. instead of at 175° F.

It will be seen from the results reported in the following Table 4 that the addition of the alkyl amino mono-

alkanols imparts improved and long-lasting vapor phase anti-rust characteristics to a variety of lubricating oils and hydraulic fluids. It is further seen that the instant mono-alkanol compounds are markedly superior to alkyl amino di-alkanols such as used in the hydraulic fluids 5 2e, 2g, 2i and 2j.

measuring the characteristics of such emulsions, is conducted by circulating the emulsion to be tested in a Vickers vane type pump, Model V-111-E10 (rated at 2 gallons per minute). This is a positive displacement vane-type hydraulic pump. The rotor has 12 steel vanes in contact with a steel ring and turns at about 1200 r.p.m.

TABLE 4.—VAPOR PHASE ANTI-RUST TEST

| Test No. | Lubricant                                                         | Wt. Percent Inhibitor        | Percent Panel Surface Rusted After—(Days) |     |     |    |    |    |     |
|----------|-------------------------------------------------------------------|------------------------------|-------------------------------------------|-----|-----|----|----|----|-----|
|          |                                                                   |                              | 3                                         | 6   | 10  | 17 | 25 | 50 | 100 |
| 1.       | Motor Oil <sup>1</sup> plus 5% H <sub>2</sub> O                   |                              | 100                                       |     |     |    |    |    |     |
| 1a.      | do <sup>1</sup>                                                   | 0.2 isopropylaminoethanol    | 3                                         | 3   | 3   | 3  | 3  | 3  | 3   |
| 1b.      | do <sup>1</sup>                                                   | 0.2 cyclohexylamine          | 50                                        | 70  | 70  | 80 | 90 |    |     |
| 1c.      | Motor Oil <sup>1</sup> plus 40% H <sub>2</sub> O                  | 0.2 isopropylaminoethanol    | 4                                         | 6   | 6   | 10 | 10 | 10 | 15  |
| 2.       | Hydraulic Fluid <sup>2</sup>                                      |                              | 100                                       |     |     |    |    |    |     |
| 2a.      | do <sup>2</sup>                                                   | 0.2 diethylaminoethanol      | 0                                         | 0   | 0   | 0  | 0  | 0  | 5   |
| 2b.      | do <sup>2</sup>                                                   | 0.2 diisopropylaminoethanol  | 4                                         | 4   | 6   | 8  | 15 | 18 | 35  |
| 2c.      | do <sup>2</sup>                                                   | 0.2 dimethylaminoethanol     | 4                                         | 4   | 4   | 4  | 6  | 7  | 7   |
| 2d.      | do <sup>2</sup>                                                   | 0.2 ethylaminoethanol        | 4                                         | 4   | 5   | 6  | 8  | 8  | 8   |
| 2e.      | do <sup>2</sup>                                                   | 0.2 isopropylaminoethanol    | 70                                        | 80  | 100 | 5  | 5  | 5  | 8   |
| 2f.      | do <sup>2</sup>                                                   | 0.2 n-butyraminoethanol      | 5                                         | 5   | 5   | 5  | 5  | 5  | 8   |
| 2g.      | do <sup>2</sup>                                                   | 0.2 butylaminoethanol        | 70                                        | 80  | 100 | 6  | 6  | 8  | 8   |
| 2h.      | do <sup>2</sup>                                                   | 0.2 methylaminoethanol       | 5                                         | 5   | 6   | 6  | 6  | 8  | 8   |
| 2i.      | do <sup>2</sup>                                                   | 0.2 methylaminoethanol       | 85                                        | 100 |     |    |    |    |     |
| 2j.      | do <sup>2</sup>                                                   | 0.2 ethylaminoethanol        | 90                                        | 100 |     |    |    |    |     |
| 2k.      | do <sup>2</sup>                                                   | 0.2 isopropylaminoethanol    | 8                                         | 8   | 8   | 8  | 8  | 8  | 8   |
| 3.       | Turbine Oil <sup>3</sup> plus 5% H <sub>2</sub> O                 |                              | 80                                        |     |     |    |    |    |     |
| 3a.      | do <sup>3</sup>                                                   | 0.3 isopropylaminoethanol    | 0                                         | 0   | 0   | 0  | 0  | 0  |     |
| 3b.      | do <sup>3</sup>                                                   | 0.3 diethylaminoethanol      | 0                                         | 0   | 0   | 0  | 0  | 0  |     |
| 3c.      | do <sup>3</sup>                                                   | 0.3 dimethylaminoethanol     | 0                                         | 0   | 0   | 0  | 0  | 1  |     |
| 3d.      | do <sup>3</sup>                                                   | 0.3 ethylaminoethanol        | 0                                         | 0   | 0   | 0  | 0  | 0  |     |
| 4.       | Premium Motor Oil <sup>4</sup> plus 5% H <sub>2</sub> O           |                              | 100                                       |     |     |    |    |    |     |
| 4a.      | do <sup>4</sup>                                                   | 0.3 isopropylaminoethanol    | 4                                         | 4   | 4   | 5  | 5  | 5  | 5   |
| 4b.      | do <sup>4</sup>                                                   | 0.3 diethylaminoethanol      | 4                                         | 5   | 6   | 6  | 10 | 10 | 10  |
| 5.       | Premium Hydraulic Oil <sup>5</sup> plus 5% added H <sub>2</sub> O |                              | 30                                        | 50  | 70  | 80 | 90 |    |     |
| 5a.      | do <sup>5</sup>                                                   | 0.3 isopropylaminoethanol    | 0                                         | 0   | 0   | 0  | 0  | 1  |     |
| 5b.      | do <sup>5</sup>                                                   | 0.3 diethylaminoethanol      | 0                                         | 0   | 0   | 0  | 0  | 0  |     |
| 5c.      | do <sup>5</sup>                                                   | 0.3 dimethylaminoethanol     | 0                                         | 0   | 0   | 0  | 0  | 0  |     |
| 5d.      | do <sup>5</sup>                                                   | 0.3 ethylaminoethanol        | 0                                         | 0   | 0   | 0  | 0  | 0  |     |
| 6.       | SAE 30 Base Oil <sup>6</sup> plus 15% H <sub>2</sub> O            |                              | 100                                       |     |     |    |    |    |     |
| 6a.      | do <sup>6</sup>                                                   | 0.3 isopropylaminoethanol    | 0                                         | 0   | 0   | 0  | 0  | 0  | 1   |
| 6b.      | do <sup>6</sup>                                                   | 0.3 diethylaminoethanol      | 0                                         | 0   | 0   | 0  | 0  | 0  | 0   |
| 6c.      | do <sup>6</sup>                                                   | 0.3 ethylaminoethanol        | 0                                         | 0   | 0   | 0  | 0  | 0  | 0   |
| 6d.      | do <sup>6</sup>                                                   | 0.3 diisopropylaminoethanol  | 12                                        | 12  | 12  | 12 | 12 | 12 | 12  |
| 6e.      | do <sup>6</sup>                                                   | 0.3 dimethylaminoethanol     | 0                                         | 0   | 0   | 0  | 0  | 0  | 0   |
| 6f.      | do <sup>6</sup>                                                   | 0.3 methylaminoethanol       | 0                                         | 0   | 0   | 0  | 0  | 0  | 0   |
| 6g.      | do <sup>6</sup>                                                   | 0.3 butylaminoethanol        | 1                                         | 1   | 1   | 1  | 1  | 2  | 2   |
| 6h.      | do <sup>6</sup>                                                   | 0.3 dimethylamino-2-propanol | 0                                         | 0   | 0   | 0  | 5  | 8  | 8   |
| 7.       | Heavy Diesel Engine Oil <sup>7</sup> plus 15% H <sub>2</sub> O    |                              | 8 100                                     |     |     |    |    |    |     |
| 7a.      | do <sup>7</sup>                                                   | 0.2 isopropylaminoethanol    | 6                                         | 8   | 6   | 6  | 6  | 6  |     |
| 7b.      | do <sup>7</sup>                                                   | 0.2 diethylaminoethanol      | 1                                         | 1   | 2   | 2  | 2  | 2  |     |
| 7c.      | do <sup>7</sup>                                                   | 0.2 ethylaminoethanol        | 4                                         | 4   | 5   | 5  | 5  | 5  |     |
| 7d.      | do <sup>7</sup>                                                   | 0.2 diisopropylaminoethanol  | 12                                        | 20  | 20  | 20 | 20 | 30 |     |
| 7e.      | do <sup>7</sup>                                                   | 0.2 dimethylaminoethanol     | 0                                         | 0   | 0   | 0  | 0  | 0  |     |
| 7f.      | do <sup>7</sup>                                                   | 0.2 methylaminoethanol       | 5                                         | 5   | 5   | 6  | 6  | 6  |     |
| 7g.      | do <sup>7</sup>                                                   | 0.2 n-butyraminoethanol      | 25                                        | 25  | 25  | 25 | 25 | 25 |     |
| 7h.      | do <sup>7</sup>                                                   | 0.2 dimethylamino-2-propanol | 3                                         | 6   | 6   | 6  | 6  | 6  |     |

<sup>1</sup> Commercial product containing cross-graded base oil of 20% 130 S.U.S. (100° F.) neutral stock, 20% solvent refined 200 S.U.S. (100° F.) neutral, 60% 100 S.U.S. (100° F.) naphthenic stock.

<sup>2</sup> Commercial hydraulic fluid of about 52% 100 S.U.S. (100° F.) naphthenic stock, about 40% water.

<sup>3</sup> Solvent refined neutral stock of 150 S.U.S. (100° F.).

<sup>4</sup> Commercial product, base oil contains about 80% solvent refined neutral stock of 130 S.U.S. (100° F.), 20% solvent refined naphthenic stock of 100 S.U.S. (100° F.).

<sup>5</sup> Commercial hydraulic oil containing 150 S.U.S. (100° F.) solvent-refined neutral paraffinic mineral oil and about 40% water.

<sup>6</sup> Oil blend consisting of 64% paraffinic solvent-refined neutral mineral oil of 200 S.U.S. (100° F.) and 36% bright stock of 2,650 S.U.S. (100° F.).

<sup>7</sup> Commercial diesel engine lubricant containing about 50% 3,300 S.U.S. (100° F.) solvent-refined coastal bright stock and 40% 520 S.U.S. (100° F.) naphthenic stock.

<sup>8</sup> 90% of panel surface rusted within 4 hours.

#### Vickers pump test

In order to determine the anti-wear properties and fluid life of the water-in-oil emulsions in addition to their vapor phase anti-rust characteristics, the emulsions were subjected to a Vickers pump test.

The Vickers pump test, which is a recognized test for 75

70 The 12 vanes and the ring are weighed before and after the test, and the difference in weight before and after is reported as total wear. The anti-rust characteristics of the fluids tested were determined by clamping the steel test panel inside the brass lid of the Vickers pump reservoir.

The results of the tests are reported in Table 5.

TABLE 5.—EFFECT OF VAPOR PHASE INHIBITORS IN VICKERS PUMP TESTS AT 1,000 P.S.I., 175° F., 2 GAL./MIN.

| Test No. | Inhibitor                      | Wt. Percent | Hours of Operation                                                                                   | Percent of Surface Rusted                                              | Total Wear, mg.                                                                   |    |
|----------|--------------------------------|-------------|------------------------------------------------------------------------------------------------------|------------------------------------------------------------------------|-----------------------------------------------------------------------------------|----|
| 1        | None                           |             | 71<br>238<br>406<br>574<br>741<br>1,006                                                              | 100<br>57<br>72<br>89<br>104<br>281                                    | 32<br>57<br>72<br>89<br>104<br>281                                                | 10 |
| 2        | Isopropyl amino ethanol        | 0.2         | 69<br>222<br>391<br>557<br>724<br>988<br>1,064<br>1,130<br>1,235<br>1,303<br>1,446<br>1,616<br>1,782 | 1<br>1<br>1<br>1<br>1<br>1<br>1<br>2<br>40<br>100<br>100<br>100<br>100 | 37<br>57<br>66<br>76<br>86<br>96<br>102<br>104<br>111<br>122<br>132<br>147<br>161 | 15 |
| 3        | Butylamine                     | 0.05        | 264<br>438<br>695<br>1,080                                                                           | 15<br>20<br>70<br>2100                                                 | 96<br>180<br>346<br>468                                                           | 25 |
| 4        | do                             | 0.07        | 260<br>340<br>980                                                                                    | 3<br>20<br>2100                                                        | 96<br>164<br>200                                                                  | 20 |
| 5        | Isopropylamine plus hexylamine | 0.1<br>0.1  | 122<br>288<br>551<br>724<br>1,365                                                                    | 0<br>0<br>5<br>60<br>2100                                              | 118<br>152<br>182<br>200<br>235                                                   | 30 |

<sup>1</sup> Commercial hydraulic fluid described in Table 1.

<sup>2</sup> Reservoir badly rusted.

It will be noted from Table 5 that the emulsion (test 2) containing the instant alkyl amino mono-alkanol compound possesses superior vapor phase anti-rust characteristics, as well as low wear rates and prolonged emulsion life. By contrast, it is seen from tests 3-5 that at the end of about 1000 test hours, emulsions containing butylamine or isopropylamine and hexylamine mixtures completely lost their useful vapor phase rust protection so that not only was the test panel badly rusted but the reservoir of the pump was also rusted. In addition, it is seen that the emulsions of these tests 3-5 possessed decidedly inferior anti-wear properties as evidenced by their high total wear values. Thus, for example, after about 1000 hours, the emulsions of tests 3 and 4 had total wear values of 468 and 200 mg. respectively, compared to 102 mg. total wear obtained with the emulsion of test 2.

#### Four-ball fatigue test

As indicated hereinabove a major drawback to the wider use of water-in-oil hydraulic fluids is their poor anti-fatigue properties. A particular advantage of the water-in-oil emulsions of this invention, however, is their improved anti-fatigue life. This is shown by the Four-Ball Fatigue Test.

According to this test three lower steel balls are allowed to spin freely in a conforming race driven by a fourth steel ball which is held firmly in the chuck of the spindle of the four-ball fatigue tester. The load employed is 294 pounds and the speed 5200 r.p.m. The test is terminated when one of the balls shows a fatigue pit which is indicated by excessive noise and vibration. This vibration actuates a vibration switch in the drive-motor electrical circuit which turns off the tester.

The longer the time period to failure the greater is the anti-fatigue qualities of the fluid tested. The results are reported in the following Table 6.

TABLE 6.—FOUR-BALL FATIGUE TEST

| Test No. |                                                    | Hours to failure |
|----------|----------------------------------------------------|------------------|
| 1        | Hydraulic fluid <sup>1</sup>                       | 19.9             |
| 2        | Hydraulic fluid plus 0.3% isopropyl amino ethanol. | 50.0             |

<sup>1</sup> Commercial hydraulic fluid containing about 52% 100 S.U.V. (100° F.) naphthenic stock, 40% water.

As can be seen from the above, the addition of isopropylamino ethanol to the hydraulic fluid increased the time period to failure from 19.9 to 50 hours thereby indicating the increased anti-fatigue qualities imparted to the emulsion.

#### Gear pump test

The improved anti-fatigue characteristics and the resulting increased pump life achieved by the use of the water-in-oil emulsions of the invention is further demonstrated by the data obtained from gear pump runs using a Commercial Shearing Model D-2 inch gear pump.

The gear pump was run to failure under 1500 p.s.i. pressure at 1200 r.p.m. at 150° F. The failure was detected by an overload device when the amperage exceeded a preset level. The results are given in the following Table 7 where it is seen that the addition of the isopropylamino ethanol lengthened the time period to failure from 165 hours (test 1) to 279 hours (test 2).

TABLE 7.—GEAR PUMP TEST

| Test No. | Composition                                        | Hours to failure |
|----------|----------------------------------------------------|------------------|
| 1        | Hydraulic fluid <sup>1</sup>                       | 165              |
| 2        | Hydraulic fluid plus 0.2% isopropyl amino ethanol. | 279              |
| 3        | Hydraulic fluid plus 0.6% isopropyl amino ethanol. | 203              |

<sup>1</sup> Commercial water-in-oil emulsion containing about 52% 100 S.U.V. (100° F.) naphthenic stock, 40% water.

The alkyl amino mono-alkanol compounds of the invention may be employed in the form of relatively pure compounds or as mixtures of different alkyl amino mono-alkanols. The amount of alkyl alkanol amines which should be used in the lubricant compositions will vary depending on such factors as the nature of the lubricant, its intended use, the presence or absence of other additives, etc. In general, from about 0.05 to about 5 weight percent, preferably from about 0.1 to about 1.0 weight percent are suitable. The use of larger amounts may in some instances be suitable depending on economic considerations.

The lubricant compositions of the invention may also contain other ingredients normally used with such compositions such as antioxidants, detergents, V.I. improvers, inhibitors, E.P. agents, pour point improvers, and in the case of water-in-oil emulsions, emulsifiers, stabilizing agents, anti-freeze agents etc.

It will, of course, be appreciated that many variations and modifications may be practiced without departing from the scope and spirit of the present invention.

Having described the invention, what I desire to secure and claim by Letters Patent is:

1. A liquid lubricant composition containing an effective amount sufficient to provide corrosion resistance thereto of a mono-alkanol compound of the formula:



where R represents an alkyl group; R' is selected from the class consisting of alkyl groups and hydrogen atoms; the sum of R+R' is equal to from 1 to about 10 carbon atoms; X is an alkylene group having from 2 to about 4

carbon atoms; and  $n$  represents an integer selected from the class consisting of 1 and 2.

2. The composition of claim 1 which contains a lubricating oil.

3. The composition of claim 1 which contains a water-in-oil emulsion.

4. A liquid lubricating composition containing a minor amount of a vapor phase anti-corrosion agent of the formula:



where R represents an alkyl group; R' is selected from the class consisting of alkyl groups and hydrogen atoms; the sum of R+R' is equal to from 1 to about 10 carbon atoms; X is an alkylene group having from 2 to about 4 carbon atoms; and n represents an integer selected from the class consisting of 1 and 2.

5. The composition of claim 4 which contains water.

6. The composition of claim 4 which contains a mineral lubricating oil.

7. The composition of claim 4 which contains a synthetic lubricating oil.

8. The composition of claim 4 which contains a water-in-oil emulsion.

9. The composition of claim 8 wherein said water-in-oil emulsion contains from about 10 to about 70% by weight of water.

10. The composition of claim 4 wherein said vapor phase anti-corrosion agent is present in an amount from about 0.05 to about 5 weight percent.

11. The composition of claim 4 wherein said vapor phase anti-corrosion agent is isopropylamino ethanol.

12. The composition of claim 4 wherein said vapor phase anti-corrosion agent is diethylamino ethanol.

13. The composition of claim 4 wherein said vapor phase anti-corrosion agent is diisopropylamino ethanol.

14. A hydraulic fluid containing from about 10 to about 70% by weight of water, a hydrocarbon oil having a Saybolt Universal viscosity at 100° F. from about 50 to about 400 seconds, and an effective amount sufficient to provide corrosion resistance thereto of a mono-alkanol compound of the formula shown in claim 4.

15. The composition of claim 4 wherein said vapor phase anti-corrosion agent is ethylamino ethanol.

16. The composition of claim 4 wherein said vapor phase anti-corrosion agent is butylamino ethanol.

17. The composition of claim 4 wherein said vapor phase anti-corrosion agent is dimethylamino ethanol.

18. A process for lubricating moving metal surfaces normally subject to vapor phase corrosion and metal fatigue wherein the said metal surfaces enclose vapor spaces in which water is present which comprises the steps of (1) incorporating into a liquid lubricating composition an effective amount sufficient to provide vapor phase corrosion resistance and anti-fatigue characteristics thereto of a compound of the formula



15

where R represents an alkyl group; R' is selected from the class consisting of alkyl groups and hydrogen atoms; the sum of R and R' is equal to from 1 to about 10 carbon atoms; X is an alkylene group having from 2 to about 4 carbon atoms; and n represents an integer selected from the class consisting of 1 and 2, and (2) introducing said liquid lubricating composition into a moving lubrication system operating under conditions normally conducive to

25 the formation of water vapor whereby the said moving metal surfaces are contacted therewith.

19. The process of claim 18 wherein the said compound is isopropylamino ethanol.

20. The process of claim 18 wherein said additive is employed in an amount from about 0.05 to about 5 weight percent.

21. The process of claim 18 wherein said liquid lubricating composition is a water-in-oil emulsion.

35

#### References Cited by the Examiner

##### UNITED STATES PATENTS

2,512,949 6/1950 Lieber ----- 252-392 X  
2,956,889 10/1960 Denman ----- 252-392 X

##### OTHER REFERENCES

"Aliphatic Nitrogen Compounds," Carbide & Carbon Chemicals Co., 1952, p. 13.

"Priminox," Rohm and Haas Co., 1959, all pages.

40

45 DANIEL E. WYMAN, Primary Examiner.

C. F. DEES, Assistant Examiner.

#### Disclaimer

3,280,029.—*Hans F. Waldmann*, Glassboro, N.J. LUBRICANT COMPOSITIONS. Patent dated Oct. 18, 1966. Disclaimer filed June 10, 1969, by the assignee, *Mobil Oil Corporation*.

Hereby enters this disclaimer to claims 1, 2, 4, 6, 7, 10 and 12 of said patent.  
[Official Gazette October 14, 1969.]

**Disclaimer**

3,280,029.—*Hans F. Waldmann*, Glassboro, N.J. LUBRICANT COMPOSITIONS. Patent dated Oct. 18, 1966. Disclaimer filed June 10, 1969, by the assignee, *Mobil Oil Corporation*.

Hereby enters this disclaimer to claims 1, 2, 4, 6, 7, 10 and 12 of said patent.  
[*Official Gazette October 14, 1969.*]